

2,847,290

## ANTI-SLAKING BUFFING COMPOSITIONS

Byron E. Marsh, Brookfield, and Richard L. Betcher, Chicago, Ill., assignors to Armour and Company, Chicago, Ill., a corporation of Illinois

No Drawing. Application April 10, 1957  
Serial No. 651,828

6 Claims. (Cl. 51—304)

This invention relates to improved buffing positions. In one of its aspects, this invention relates to lime buffing bars having improved anti-slaking properties.

Conventional buffing compositions in use for buffing nickel, nickel alloys, copper, brass, zinc, aluminum, etc., have proven unsatisfactory in many respects. Such compositions usually contain lime and are used in the form of bars. In use these bars are rubbed against the buffing wheel and the abrasive is applied to the wheel by melting binder brought about through the heat of friction.

The production of lime compositions has caused problems in the buffing industry for years. An insoluble lime soap is often formed when mixing the calcium and magnesium oxide abrasives and the fatty acid binder in the presence of moisture. When this occurs in the kettle it is necessary to break the hard cellular soap into pieces that can be usually removed, since heat will only char the soap, not melt it. In addition to soap formation, the most pressing problem from a consumer point of view is slaking. This term is used to describe the hydration of the hard oxides to the soft hydroxides in the presence of atmospheric moisture and normally takes place within one to three weeks after formation of the lime bar unless an airtight container is used for storage of the composition. As hydration occurs the slaked lime reacts with the fatty acid binder and the bar flakes and eventually crumbles. In this condition of course it cannot be used in buffing operations. The industry has alleviated the problem somewhat by the use of quality controlled materials, close supervision in manufacture, and the use of expensive airtight containers similar to the vacuum sealed food containers. However, even with these precautions, storage of lime bars for any length of time is not practiced and orders are filled only when received. It is obvious, therefore, that there exists a need for an anti-slaking additive in lime buffing compositions.

In accordance with the present invention we have provided an anti-slaking additive for lime buffing compositions which enables buffing bar compounders to produce bars for stock, which they have been unable to do before because of the short storage life. This makes possible easier production scheduling and the preparation of larger sized batches. Also, it enables the use of a cheap paper container in place of an expensive airtight metal container or foil.

Our anti-slaking additives are N-aliphatic-trimethylene diamines which can be represented by the structural formula  $RNHCH_2CH_2CH_2NH_2$  wherein R is an aliphatic hydrocarbon radical containing from 8 to 22 carbon atoms. Examples of aliphatic radicals coming within the definition of R include octyl, decyl, dodecyl, tetradecyl, hexadecyl, octadecyl, octadecenyl, octadecadienyl, octadecatrienyl, and statistical mixtures of the foregoing radicals as are contained in naturally occurring oils and fats such as tallow, soybean oil, coconut oil, and the like. The mixture of aliphatic hydrocarbon radicals contained in tallow is comprised of approximately 45% by weight of octadecenyl, 25% octadecyl, and 30% hexadecyl radi-

2  
cals. Examples of preferred anti-slaking additives include N-tallow-trimethylene diamine, N-octadecyl-trimethylene diamine and N-hexadecyl-trimethylene diamine.

The improved anti-slaking by lime buffering compositions of the present invention contain from about 65 to 80% by weight of lime, such as Vienna lime, as the abrasive element, from about 12 to 18% of a saturated fatty acid having a titer of at least 40° C., preferably having an iodine value not in excess of 7.0, from about 12 to 18% of an animal or vegetable oil glyceride, and from about 1.5 to about 5.0%, preferably about 5.0% of our anti-slaking additive as described above. If desired, the abrasive element can contain in addition to the lime conventional materials such as emery, silicon carbide, tripoli, or the like.

The buffering compositions of the present invention can be prepared by blending together the anti-slaking additives, saturated fatty acid, and animal oil at a temperature of about 190° F. after which the abrasive material is added to the molten material with mixing until a smooth mixture is obtained. The molten paste can then be put into forms and allowed to cool and harden.

The following example will illustrate this invention in the manner in which it may be practiced, but it is to be understood that this example is not to be construed as unduly limiting:

*Example*

Three series of two buffering bars, A and B, were prepared and observed under different storage conditions for slaking. The bars were prepared in the manner described above. Bar A contained 15% by weight of stearic acid having a titer of 54° C. and an iodine value of 7, 15% acidless tallow and 70% lime composed of 50% CaO and 50% MgO. Bar B contained 15% by weight of stearic acid having a titer of 54° C. and an iodine value of 7, 15% acidless tallow, 5% N-tallow-trimethylene diamine and 65% lime composed of 50% CaO and 50% MgO. Each of the bars were stored in unsealed containers.

One group of bars was stored in a humidity cabinet of 110° F. and 93% relative humidity. Bar A slaked in less than 72 hours. Bar B showed no evidence of slaking after 96 hours.

Another group of bars was stored in an air oven at 160° F. Bar A slaked in 6 days. Bar B showed no evidence of slaking after 38 days.

Still another group was stored under ordinary conditions, but unwrapped. Bar A slaked after 14 days. Bar B showed slaking on the surface only after 38 days of storage.

While this invention has been described and exemplified in terms of its preferred embodiments, those skilled in the art will appreciate that modifications can be made without departing from the spirit and scope of the invention.

We claim:

1. An improved lime buffering composition containing as an anti-slaking additive from about 1.5% to about 5.0% by weight of a compound having the formula  $RNHCH_2CH_2CH_2NH_2$  wherein R is an aliphatic hydrocarbon radical having from 8 to 22 carbon atoms.
2. An improved lime buffering composition containing as an anti-slaking additive from about 1.5 to about 5.0 weight percent of N-tallow-trimethylene diamine.
3. An improved lime buffering composition containing as an anti-slaking additive about 5.0% by weight of N-tallow-trimethylene diamine.
4. A lime buffering composition consisting of about 65 to 80% by weight of Vienna lime, about 12 to 18% of a saturated fatty acid having a titer of at least 40° C., from about 12 to about 18% of tallow and 1.5 to about

5.0% by weight of a compound having the formula  $RNHCH_2CH_2CH_2NH_2$  wherein R is an aliphatic hydrocarbon radical having from 8 to 22 carbon atoms.

5. A composition according to claim 4 wherein the saturated fatty acid is stearic acid and R is a mixture of aliphatic hydrocarbon radicals as contained in tallow.

6. A lime buffering composition consisting of about 65% by weight of Vienna lime, 15% stearic acid, 15% acidless tallow, and 5.0% of N-tallow-trimethylene diamine.

## References Cited in the file of this patent

## UNITED STATES PATENTS

|           |           |       |                |
|-----------|-----------|-------|----------------|
| 2,078,876 | Hennessey | ----- | Apr. 27, 1937  |
| 2,417,800 | Weisser   | ----- | Mar. 18, 1947  |
| 2,482,667 | Gray      | ----- | Sept. 20, 1949 |
| 2,606,829 | Chester   | ----- | Aug. 12, 1952  |
| 2,642,348 | Stier     | ----- | June 16, 1953  |